

Patented Nov. 13, 1951

2,574,806

# UNITED STATES PATENT OFFICE

2,574,806

## COMPOSITIONS AND PROCESSES FOR PRINTING ORGANIC DERIVATIVES OF CELLULOSE USING A MIXTURE OF FOUR SWELLING AGENTS

Alexis Wiazmitinow and Henk Goorhuis, Basel,  
Switzerland, assignors to Sandoz A. G., Basel,  
Switzerland, a Swiss firm

No Drawing. Application May 9, 1949, Serial No.  
92,246. In Switzerland May 14, 1948

10 Claims. (Cl. 8—63)

1

The present invention relates to a new and improved process for the dyeing and printing of organic derivatives of cellulose allowing dyestuffs of various constitution to be fixed on the said cellulose derivatives without use of a steaming operation. Until now different processes for the fixation of water-soluble acid dyestuffs on cellulose esters and ethers have been suggested. In order to obtain this result it has been proposed to add to the dyebaths or printing pastes compounds, such as aliphatic carboxylic acids or alcohols, esters of organic acids, such as ethyl acetate, acetone and the like, and furthermore swelling agents, such as the salts of thiocyanic acid, phenols and the like. Generally the fixation of the dyestuffs is realized by subjecting the printed material to a steaming operation. It is further known that by the use of an increased quantity of sodium thiocyanate in the presence of methanol and acetic acid, acid dyestuffs may be printed on acetate silk and fixed by a simple drying of the printed material. But this fixation is not a quantitative one and the strong swelling action of the sodium thiocyanate can easily provoke a destruction of the fibre and of the acid azo dyestuff which becomes reduced by the sodium thiocyanate.

It has now been found that organic derivatives of cellulose can be dyed or printed in shades fast to washing by means of water-soluble dyestuffs which have no or a poor affinity to such cellulose derivatives, when during the dyeing or printing of such fibres padding baths or printing pastes are used which contain besides the said dyestuffs and conventional stretching and diluting agents at least one water-soluble salt of thiocyanic acid, a swelling agent of the general formula



wherein X stands for O, S or NH, a volatile aliphatic carboxylic acid and an aliphatic hydroxylated compound. The quantity of the salt of the thiocyanic acid which is used according to the present invention may be for instance about 3% in the case of sodium thiocyanate, calculated on the weight of the dye-bath or printing paste.

As swelling agents falling within the scope of the above general formula, use may be made of urea, thiourea and guanidine.

As volatile aliphatic carboxylic acids we use preferably formic and acetic acid and as aliphatic hydroxylated compounds glycols, polyglycols, their ethers containing at least one free hydroxy

group, thioglycols and similar compounds may be employed.

The fixation of the dyes is realized by a simple drying of the dyed or printed material at a temperature of for example 40—50° C. After drying, the material is preferably first washed with cold water, then soaped at 60° C. and finished in the conventional manner.

The present invention is particularly suitable for printing and dyeing by padding acetate silk. If it is applied to mixed fabrics containing for example acetate and pure silk it is advisable to have a steam operation to follow the printing or padding operation in order to effect the fixation on both fibres that is to say on the cellulose acetate and also the silk fibre.

The following examples, without being limitative, show how the present invention can be carried out.

### EXAMPLE 1

A piece of acetate silk is padded in a bath of the following composition:

|                                                    |
|----------------------------------------------------|
| 7.5 grams of acid Violet 4BNS (Colour Index N 806) |
| 25 562.5 grams of water                            |
| 100.0 grams of tragacanth thickening 60/1000       |
| 100.0 grams of ethylene glycol                     |
| HO—CH <sub>2</sub> —CH <sub>2</sub> —OH            |
| 30 100.0 grams of thiourea                         |
| 30.0 grams of ammonium thiocyanate                 |
| 100.0 grams of acetic acid conc. 100%              |

1000.0 grams

35 The padded piece is dried at 40—50° C., rinsed cold and soaped at 60° C. The piece dyed in this manner has a violet colour which is fast to washing and may be soaped at boiling temperature without bleeding.

### EXAMPLE 2

Acetate silk is printed with any one of the following printing recipes:

45 (a)

|                                                                             |
|-----------------------------------------------------------------------------|
| 7.5 grams of Xylene Fast Green B (Colour Index 777)                         |
| 162.5 grams of water                                                        |
| 500.0 grams of tragacanth thickening 60/1000                                |
| 100.0 grams of ethylene thioglycol                                          |
| HO—H <sub>2</sub> C—H <sub>2</sub> C—S—CH <sub>2</sub> —CH <sub>2</sub> —OH |
| 100.0 grams of urea                                                         |
| 30.0 grams of ammonium thiocyanate                                          |
| 100.0 grams of acetic acid conc. 100%                                       |

1000.0 grams

3  
(b)

15.0 grams of Azo Rhodine 2G (Colour Index 40)  
 155.0 grams of water  
 500.0 grams of tragacanth thickening 60/1000  
 100.0 grams of ethylene thiodiglycol  
 100.0 grams of thiourea  
 30.0 grams of ammonium thiocyanate  
 100.0 grams of formic acid 80%  
 1000.0 grams

(c)

25.0 grams of Brilliant Sulphon Red B (Colour Index 41)  
 145.0 grams of water  
 500.0 grams of tragacanth thickening 60/1000  
 100.0 grams of ethylene thiodiglycol  
 100.0 grams of thiourea  
 30.0 grams of ammonium thiocyanate  
 100.0 grams of acetic acid conc. 100%  
 1000.0 grams

(d)

15.0 grams of Xylene Fast Blue AE (Colour Index 974)  
 155.0 grams of water  
 500.0 grams of tragacanth thickening 60/1000  
 100.0 grams of diethyleneglycol-monobutylether  
 $\text{CH}_3\text{-CH}_2\text{-CH}_2\text{-CH}_2\text{-O-CH}_2\text{-CH}_2\text{-O-CH}_2\text{-CH}_2\text{-OH}$   
 100.0 grams of thiourea  
 30.0 grams of ammonium thiocyanate  
 100.0 grams of acetic acid conc. 100%  
 1000.0 grams

(e)

15.0 grams of Xylene Light Yellow R (Colour Index 736)  
 145.0 grams of water  
 500.0 grams of tragacanth thickening 60/1000  
 100.0 grams of ethylene thiodiglycol  
 100.0 grams of thiourea  
 40.0 grams of zinc thiocyanate  
 100.0 grams of acetic acid conc. 100%  
 1000.0 grams

(f)

7.5 grams of Xylene Red B (Colour Index 863)  
 152.5 grams of water  
 500.0 grams of tragacanth thickening 60/1000  
 100.0 grams of ethylene thiodiglycol  
 100.0 grams of thiourea  
 40.0 grams of potassium thiocyanate  
 100.0 grams of acetic acid conc. 100%  
 1000.0 grams

(g)

15.0 grams of Xylene Blue AS (Colour Index 771)  
 140.0 grams of water  
 500.0 grams of tragacanth thickening 60/1000  
 100.0 grams of thiourea  
 100.0 grams of ethylene thiodiglycol  
 45.0 grams of barium thiocyanate 2 aq.  
 100.0 grams of acetic acid conc. 100%  
 1000.0 grams

4  
(h)

7.5 grams of Xylene Red B (Colour Index 863)  
 152.5 grams of water  
 500.0 grams of tragacanth thickening 60/1000  
 5 100.0 grams of ethylene thiodiglycol  
 100.0 grams of thiourea  
 20.0 grams of potassium thiocyanate  
 20.0 grams of sodium thiocyanate  
 100.0 grams of acetic acid conc. 100%  
 1000.0 grams

The printed material is dried at 40-50° C., rinsed with cold water and soaped at 60° C. The material printed in this way may be soaped at boiling temperature without bleeding.

## EXAMPLE 3

A printing paste containing  
 20 12.0 grams of Alizarine Light Green GS (Colour Index 1201)  
 348.0 grams of water  
 500.0 grams of tragacanth thickening 60/1000  
 50.0 grams of ethylene thiodiglycol  
 25 50.0 grams of thiourea  
 30.0 grams of ammonium thiocyanate  
 10.0 grams of acetic acid conc. 100%  
 1000.0 grams

30 is printed on a mixed fabric containing acetate silk and natural silk, whereupon the printed piece is dried at a temperature of 40-50° C., steamed for 5 minutes at 101° C., rinsed with cold water and soaped at 60° C. The print obtained in this way is fast to washing, the acetate silk fibres having not been damaged by the swelling agent present in the printing paste.

## EXAMPLE 4

40 Acetate silk is printed with any one of the following printing pastes of the following composition:

(a)  
 45 10.0 grams of Auramine O (Colour Index 655)  
 100.0 grams of ethylene thiodiglycol  
 160.0 cc. of water  
 500.0 grams of tragacanth thickening 60/1000  
 100.0 grams of thiourea  
 50 30.0 grams of ammonium thiocyanate  
 100.0 grams of acetic acid conc. 100%  
 1000.0 grams

(b)  
 55 5.0 grams of Rhodamine B (Colour Index 749)  
 100.0 grams of ethylene glycol  
 165.0 cc. of water  
 500.0 grams of tragacanth thickening 60/1000  
 100.0 grams of thiourea  
 60 30.0 grams of ammonium thiocyanate  
 100.0 grams of acetic acid conc. 100%  
 1000.0 grams

(c)  
 65 15.0 grams of Chlorantine Light Yellow 4GL (Colour Index No. 346)  
 100.0 grams of ethylene thiodiglycol  
 155.0 cc. of water  
 70 500.0 grams of tragacanth thickening 60/1000  
 100.0 grams of thiourea  
 30.0 grams of ammonium thiocyanate  
 100.0 grams of acetic acid conc. 100%  
 1000.0 grams

75 1000.0 grams

30.0 grams of Prune pur (Colour Index No. 893)  
 40.0 grams of Tetracarnit  
 100.0 grams of ethylene thiodiglycol  
 100.0 cc. of water  
 500.0 grams of tragacanth thickening 60/1000  
 100.0 grams of thiourea  
 30.0 grams of ammonium thiocyanate  
 100.0 grams of acetic acid conc. 100%  


---

 1000.0 grams

The printed materials are dried at a temperature of 40-50° C., rinsed with cold water and soaped at 60° C., whereupon the materials are once more rinsed. The prints obtained in this manner are fast to soaping.

What we claim is:

1. A process for producing prints, which are fast to soaping, on textile materials composed of cellulose acetate, with a water-soluble dyestuff having substantially no affinity for cellulose acetate, which comprises the steps of applying to the said material an aqueous printing composition containing the said dyestuff, a thickening agent, 2-5% by weight of at least one water-soluble salt of thiocyanic acid, 8-12% by weight of a lower aliphatic carboxylic acid, 8-12% by weight of a swelling agent selected from the group consisting of urea, thiourea and guanidine, and 9-15% by weight of a member selected from the group consisting of ethylene glycol, ethylene thiodiglycol and diethylene glycol monobutyl ether, fixing the dye onto the thus-treated material by subjecting the latter to a simple heating operation, whereby the material is dried and the dye fixed thereon without the necessity of steaming, and then subjecting the dried material to a treatment with a warm soaping solution.

2. A process for producing prints, which are fast to soaping, on textile material composed of cellulose acetate, with a water-soluble acid dyestuff having substantially no affinity for cellulose acetate, which comprises the steps of applying to the said material an aqueous printing composition containing the said dyestuff, a thickening agent, 2-5% by weight of at least one water-soluble salt of thiocyanic acid, 8-12% by weight of a lower aliphatic carboxylic acid, 8-12% by weight of a swelling agent selected from the group consisting of urea, thiourea and guanidine, and 9-15% by weight of a member selected from the group consisting of ethylene glycol, ethylene thiodiglycol and diethylene glycol monobutyl ether, fixing the dye onto the thus-treated material by subjecting the latter to a simple heating operation, whereby the material is dried and the dye fixed thereon without the necessity of steaming, and then subjecting the dried material to a treatment with a warm soaping solution.

3. A process for producing prints, which are fast to soaping, on textile material composed of cellulose acetate, with a water-soluble basic dyestuff having substantially no affinity for cellulose acetate, which comprises the steps of applying to the said material an aqueous printing composition containing the said dyestuff, a thickening agent, 2-5% by weight of at least one water-soluble salt of thiocyanic acid, 8-12% by weight of a lower aliphatic carboxylic acid, 8-12% by weight of a swelling agent selected from the group consisting of urea, thiourea and guanidine, and 9-15% by weight of a member selected from the group consisting of ethylene glycol, ethylene

thiodiglycol and diethylene glycol monobutyl ether, fixing the dye onto the thus-treated material by subjecting the latter to a simple heating operation, whereby the material is dried and the dye fixed thereon without the necessity of steaming, and then subjecting the dried material to a treatment with a warm soaping solution.

4. A process for producing prints, which are fast to soaping, on textile material composed of cellulose acetate, with a water-soluble substantive dyestuff having substantially no affinity for cellulose acetate, which comprises the steps of applying to the said material an aqueous printing composition containing the said dyestuff, a thickening agent, 2-5% by weight of at least one water-soluble salt of thiocyanic acid, 8-12% by weight of a lower aliphatic carboxylic acid, 8-12% by weight of a swelling agent selected from the group consisting of urea, thiourea and guanidine, and 9-15% by weight of a member selected from the group consisting of ethylene glycol, ethylene thiodiglycol and diethylene glycol monobutyl ether, fixing the dye onto the thus-treated material by subjecting the latter to a simple heating operation, whereby the material is dried and the dye fixed thereon without the necessity of steaming, and then subjecting the dried material to a treatment with a warm soaping solution.

5. A process for producing prints, which are fast to soaping, on textile material composed of cellulose acetate, with a water-soluble mordant dyestuff having substantially no affinity for cellulose acetate, which comprises the steps of applying to the said material an aqueous printing composition containing the said dyestuff, a thickening agent, 2-5% by weight of at least one water-soluble salt of thiocyanic acid, 8-12% by weight of a lower aliphatic carboxylic acid, 8-12% by weight of a swelling agent selected from the group consisting of urea, thiourea and guanidine, and 9-15% by weight of a member selected from the group consisting of ethylene glycol, ethylene thiodiglycol and diethylene glycol monobutyl ether, fixing the dye onto the thus-treated material by subjecting the latter to a simple heating operation, whereby the material is dried and the dye fixed thereon without the necessity of steaming, and then subjecting the dried material to a treatment with a warm soaping solution.

6. A textile printing composition for the production of prints, which are fast to soaping, on textile material composed of cellulose acetate, said composition consisting essentially of water, a water-soluble dyestuff having substantially no affinity for cellulose acetate, a thickening agent, 2-5% by weight of at least one water-soluble salt of thiocyanic acid, 8-12% by weight of a lower aliphatic carboxylic acid, 8-12% by weight of a swelling agent selected from the group consisting of urea, thiourea and guanidine, and 9-15% by weight of a member selected from the group consisting of ethylene glycol, ethylene thiodiglycol and diethylene glycol monobutyl ether, whereby the desired prints which are fast to soaping may be produced without the necessity of subjecting the printed material to a steaming operation.

7. A textile printing composition for the production of prints, which are fast to soaping, on textile material composed of cellulose acetate, said composition consisting essentially of water, a water-soluble acid dyestuff having substantially no affinity for cellulose acetate, a thickening agent, 2-5% by weight of at least one water-soluble salt of thiocyanic acid, 8-12% by weight of a lower aliphatic carboxylic acid, 8-12% by weight of a member selected from the group consisting of ethylene glycol, ethylene thiodiglycol and diethylene glycol monobutyl ether, whereby the desired prints which are fast to soaping may be produced without the necessity of subjecting the printed material to a steaming operation.

weight of a swelling agent selected from the group consisting of urea, thiourea and guanidine, and 9-15% by weight of a member selected from the group consisting of ethylene glycol, ethylene thioglycol and diethylene glycol monobutyl ether, whereby the desired prints which are fast to soaping may be produced without the necessity of subjecting the printed material to a steaming operation.

8. A textile printing composition for the production of prints, which are fast to soaping, on textile material composed of cellulose acetate, said composition consisting essentially of water, a water-soluble basic dyestuff having substantially no affinity for cellulose acetate, a thickening agent, 2-5% by weight of at least one water-soluble salt of thiocyanic acid, 8-12% by weight of a lower aliphatic carboxylic acid, 8-12% by weight of a swelling agent selected from the group consisting of urea, thiourea and guanidine, and 9-15% by weight of a member selected from the group consisting of ethylene glycol, ethylene thioglycol and diethylene glycol monobutyl ether, whereby the desired prints which are fast to soaping may be produced without the necessity of subjecting the printed material to a steaming operation.

9. A textile printing composition for the production of prints, which are fast to soaping, on textile material composed of cellulose acetate, said composition consisting essentially of water, a water-soluble substantive dyestuff having substantially no affinity for cellulose acetate, a thickening agent, 2-5% by weight of at least one water-soluble salt of thiocyanic acid, 8-12% by weight of a lower aliphatic carboxylic acid, 8-12% by weight of a swelling agent selected from the group consisting of urea, thiourea and guanidine, and 9-15% by weight of a member selected from the group consisting of ethylene glycol, ethylene thioglycol and diethylene glycol monobutyl ether, whereby the desired prints which are fast

10  
15  
20

to soaping may be produced without the necessity of subjecting the printed material to a steaming operation.

10. A textile printing composition for the production of prints, which are fast to soaping, on textile material composed of cellulose acetate, said composition consisting essentially of water, a water-soluble mordant dyestuff having substantially no affinity for cellulose acetate, a thickening agent, 2-5% by weight of at least one water-soluble salt of thiocyanic acid, 8-12% by weight of a lower aliphatic carboxylic acid, 8-12% by weight of a swelling agent selected from the group consisting of urea, thiourea and guanidine, and 9-15% by weight of a member selected from the group consisting of ethylene glycol, ethylene thioglycol and diethylene glycol monobutyl ether, whereby the desired prints which are fast to soaping may be produced without the necessity of subjecting the printed material to a steaming operation.

ALEXIS WIAZMITINOW.  
HENK GOORHUIS.

#### REFERENCES CITED

The following references are of record in the file of this patent:

#### UNITED STATES PATENTS

| Number    | Name        | Date          |
|-----------|-------------|---------------|
| 1,968,855 | Rivat ----- | Aug. 7, 1934  |
| 2,428,836 | Croft ----- | Oct. 14, 1947 |

#### FOREIGN PATENTS

| Number  | Country             | Date          |
|---------|---------------------|---------------|
| 285,942 | Great Britain ----- | Feb. 23, 1928 |
| 595,344 | Great Britain ----- | Dec. 2, 1947  |
| 376,797 | Great Britain ----- | June 11, 1932 |
| 375,313 | Great Britain ----- | June 13, 1932 |

#### OTHER REFERENCES

Rayon Textile Mo. for March 1948, page 90.